



US005747208A

# United States Patent [19]

Ueda

[11] Patent Number: 5,747,208

[45] Date of Patent: May 5, 1998

[54] **METHOD OF USING PHOTORESITIVE MEMBER COMPRISING THICK PHOTORESITIVE LAYER HAVING A SPECIFIED MOBILITY**

[75] Inventor: **Hideaki Ueda**, Kishiwada, Japan

[73] Assignee: **Minolta Co., Ltd.**, Osaka, Japan

[21] Appl. No.: **908,610**

[22] Filed: **Aug. 8, 1997**

## Related U.S. Application Data

[60] Continuation of Ser. No. 650,554, May 20, 1996, abandoned, which is a division of Ser. No. 418,900, Apr. 7, 1995, abandoned, which is a continuation of Ser. No. 171,447, Dec. 22, 1993, abandoned.

## Foreign Application Priority Data

Dec. 28, 1992 [JP] Japan ..... 4-348453  
Dec. 1, 1993 [JP] Japan ..... 5-301987

[51] Int. Cl. <sup>6</sup> ..... G03G 13/06; G03G 5/047

[52] U.S. Cl. ..... 430/97; 430/58

[58] Field of Search ..... 430/58, 69, 126,  
430/97

## References Cited

### U.S. PATENT DOCUMENTS

|           |         |                  |       |        |
|-----------|---------|------------------|-------|--------|
| 4,346,157 | 8/1982  | Kakuta et al.    | ..... | 430/58 |
| 4,670,369 | 6/1987  | Nakagawa et al.  | ..... | 430/57 |
| 4,702,981 | 10/1987 | Matsumoto et al. | ..... | 430/69 |
| 4,956,256 | 9/1990  | Ohtsuka et al.   | ..... | 430/96 |
| 5,120,627 | 6/1992  | Nozomi et al.    | ..... | 430/59 |
| 5,173,384 | 12/1992 | Otsuka           | ..... | 430/59 |
| 5,294,509 | 3/1994  | Ashiya et al.    | ..... | 430/58 |
| 5,316,880 | 5/1994  | Pai et al.       | ..... | 430/58 |
| 5,328,790 | 7/1994  | Asano et al.     | ..... | 430/65 |
| 5,376,485 | 12/1994 | Yoshihara        | ..... | 430/58 |

5,397,395 3/1995 Sano et al. ..... 118/718  
5,532,101 7/1996 Nozawa et al. ..... 430/126

## FOREIGN PATENT DOCUMENTS

2-46937 11/1990 Japan .  
4-220651 8/1992 Japan .

## OTHER PUBLICATIONS

Diamond, Arthur S. (editor). *Handbook of Imaging Materials*. New York: Marcel-Dekker, Inc. pp. 160-163, 406-411, 1991.

IBM Engineering Specification 890350. Mar. 1970.

Diamond, Arthur S. (1991) *Handbook of Imaging Materials*. New York: Marcel-Dekker, Inc. pp. 387-392, 427-434, 439.

Primary Examiner—Christopher D. Rodee  
Attorney, Agent, or Firm—Burns, Doane, Swecker & Mathis, LLP

[57]

## ABSTRACT

The present invention provides a laminated-type photosensitive member comprising a photosensitive layer which is comprised of

a charge generating layer containing an organic charge generating material and

a charge transporting layer having a thickness of at least 27  $\mu$ m and containing an organic charge transporting material

on an electrically conductive cylindrical substrate having a small drum size.

a mobility ( $\mu$ ) of electrical charges in the charge transporting layer has a specified value. The laminated-type photosensitive member can be applied to an image-forming process in which electrostatic latent images are formed at the identical position of the photosensitive member at a 0.5 or less second interval.

13 Claims, 1 Drawing Sheet

Fig. 1



**METHOD OF USING PHOTORESISTIVE  
MEMBER COMPRISING THICK  
PHOTORESISTIVE LAYER HAVING A  
SPECIFIED MOBILITY**

This application is a continuation of application Ser. No. 08/650,554, filed May 20, 1996 abandoned, which is a divisional of application Ser. No. 08/418,900, filed Apr. 7, 1995 abandoned, which is a continuation of application Ser. No. 08/171,447, filed Dec. 22, 1993 abandoned.

**BACKGROUND OF THE INVENTION**

**1. Field of the Invention**

The present invention relates to a photosensitive member of a laminated-type having a charge generating layer and a charge transporting layer, in particular to a photosensitive member having a thick charge transporting layer, which is excellent in wear resistance and electrical characteristics.

**2. Description of the Prior Art**

Known photosensitive materials for forming a photosensitive layer include inorganic photoconductive materials such as selenium, cadmium sulfide or zinc oxide. These photosensitive materials have many advantages such as low loss of charges in the dark, an electrical charge which can be rapidly dissipated with irradiation of light and the like. However, they have disadvantages. For example, a photosensitive member based on selenium is difficult to produce, has high production costs and is difficult to handle due to inadequate resistivity to heat or mechanical impact. A photosensitive member based on cadmium sulfide has defects such as its unstable sensitivity in a highly humid environment and loss of stability with time because of the deterioration of dyestuffs, added as sensitizer, by corona charge and fading with exposure. These photosensitive members also have a problem from the viewpoint of safety.

Many kinds of organic photoconductive materials such as polyvinylcarbazole and the similar compounds have been proposed for forming an organic photosensitive layer. These organic photoconductive materials have superior film forming properties, are light in weight, etc., but inferior in sensitivity, durability and environmental stability compared to the aforementioned inorganic photoconductive materials.

Various studies and developments have been in progress to overcome the above noted defects and problems. A function-divided organic photosensitive member of a laminated or a dispersed type has been proposed, in which a charge generating function and a charge transporting function are shared by different compounds. In usual, a photosensitive layer in the function-divided photosensitive member of the laminated type is composed of a charge generating layer containing an organic charge-generating material, a charge transporting layer containing an organic charge-transporting material and a binder resin. A photosensitive layer in the function-divided photosensitive member of the dispersion-type is composed of an organic charge-generating material and an organic charge-transporting material which are dispersed in a binder resin.

Such a function-divided organic photosensitive member can display performances excellent in electrophotographic properties such as chargeability, sensitivity, residual potential, durability with respect to copy and repetition, because most adequate materials can be selected from various materials. Moreover, function-divided photosensitive members have high productivity and low costs, since they can be prepared by coating, and suitably selected charge generating materials can freely control a region of photosensitive wavelength.

However, the organic photosensitive member is generally poor in mechanical strength and durability compared to the inorganic photosensitive member. A thickness of the organic photosensitive member decreases with its friction against toner, paper, a cleaning member and other similar loads in the copying machine. A layer-decreasing degree caused by wear depends on materials and mechanical systems, but generally it is 0.2-1  $\mu\text{m}$  after 10,000 times of copy. The decrease of the layer-thickness causes the deterioration of chargeability. When the deterioration is beyond tolerance limits, the lifetime of the photosensitive member is over. As a result, the organic photosensitive member is poor in resistance to copy.

Moreover a system speed of a copying machine has been made high recently. A load on a photosensitive member is so severe that the wear of the photosensitive member has been a serious problem.

Therefore, it has been developed and researched that a charge transporting layer in a photosensitive layer of a laminate-type is made thick in order to improve durability and to make the lifetime of the photosensitive member long.

However when a thickness of the charge transporting layer is merely made thick, it is true that the lifetime of the photosensitive member becomes long. However the increase of the layer thickness causes deterioration of electrical properties and accumulation of electrical charges, resulting in lowering of sensitivity. Particularly, in a photosensitive member having a small diameter of at most 50  $\text{mm}\Phi$ , the above tendency is more remarkable. Because when the photosensitive member having a small diameter is used repeatedly, electrostatic latent images are formed on an identical position in a short time, it is hard to quench generated charge carriers completely by an erasing light by the time of the next charging process. As a result, electrical carriers remain in the charge transporting layer or the charge generating layer to cause the increase of residual potential and the lowering of surface potential. Accordingly the thicker the transporting layer is, or the higher the system speed is by use of a small size photosensitive member, the higher mobility is required in the charge transporting layer and the charge generating layer in order to quench the surface charges in a short time.

**SUMMARY OF THE INVENTION**

The object of the present invention is to provide a laminated-type organic photosensitive member having a thick charge transporting layer of at least 27  $\mu\text{m}$ , which is thicker than a conventional charge transporting layer of 10 to 20  $\mu\text{m}$ .

The photosensitive member of the present invention has high sensitivity, the electrical characteristics are stable even after repetition use and an increase of residual potential is low in spite of such a thick charge transporting layer.

The present invention relates to a laminated-type photosensitive member comprising a photosensitive layer which is comprised of

a charge generating layer containing an organic charge generating material and

a charge transporting layer having a thickness of at least 27  $\mu\text{m}$  and containing an organic charge transporting material

on an electrically conductive cylindrical substrate having a small drum size.

a mobility ( $\mu$ ) of electrical charges in the charge transporting layer has a specified value. The laminated-type

photosensitive member can be applied to an image-forming process in which electrostatic latent images are formed at the identical position of the photosensitive member at a 0.5 or less second interval.

#### BRIEF DESCRIPTION OF THE DRAWINGS

FIG. 1 is a schematic view of a tester for a photosensitive member.

#### DETAILED DESCRIPTION OF THE INVENTION

The present invention relates to a photosensitive member having a thick charge transporting layer compared to a conventional photosensitive layer, which can be prevented from accumulation of electrical charges in a charge generating layer and a charge transporting layer, deterioration of sensitivity and increase of residual potential.

The present invention has accomplished the above object by forming a charge generating layer and a thick charge transporting layer having a specified mobility on an electrically conductive substrate having a small diameter.

The mobility ( $\mu$ ) in this invention represents a moving speed of charge carriers in the charge transporting layer or the charge generating layer. The larger the mobility is, the higher the moving speed of the electrical charges is. The mobility has a close connection with the accumulation of electrical charges.

The mobility is obtained from a transit-time on the basis of signals sent by Time of Flight Method (TOF), in which a charge transporting layer and a charge generating layer are formed on a NESA glass and gold is sputtered to form an electrode on the surface, followed by irradiation of a nitrogen laser of 337 nm wavelength at a pulse interval of 5 nsec through the NESA glass at 25°C.

In the present invention, the charge transporting layer is made thick to improve durability and the mobility in the transporting layer is adjusted within a specified range to prevent accumulation of electrical charges in the charge transporting layer. Thereby the lowering of chargeability and the increase of residual potential can be prevented.

In the formula  $\log \mu = A \times E^{1/2} + B$  [I], the letters A and B can be determined as follows: a linear relationship between mobility ( $\mu$ ) and  $E^{1/2}$  is obtained and the letter A represents an inclination of the linear line and the letter B represents an ordinate axis crossing point of the linear line.

When the value of A is 0.11 or less, the photosensitive member depends little on a strength of electric field and the increasing change of an end portion of light-decay curve under a low electric field can be suppressed even after repetition use.

When the value of B is -5.9 or more, a sensitivity change is small at a low temperature. A layer can be made thick and the increase of a residual potential and the lowering of an initial surface potential can be suppressed. When the electrically conductive substrate having a small size is used and a copying speed is made high, it is more preferable that the value of A is 0.1 or less and that the value of B is -5 or more.

Further, a mobility ( $\mu$ ) and a space charge density (N) in the charge generating layer may be adjusted within a specified range in the present invention. Thereby charge carriers generated by light irradiation can be effectively prevented from accumulating in the charge generating layer with repetition use.

In particular, more stable charging properties can be given when the mobility is adjusted to  $1 \times 10^{-8} \text{ cm}^2/\text{V.sec}$  or more.

preferably  $5 \times 10^{-3} \text{ cm}^2/\text{V.sec}$  under the electric field of  $5 \times 10^{-5} \text{ V/cm}$  and the space charge density is adjusted to  $1 \times 10^{16} \text{ cm}^{-3}$  or less.

The space charge density (N) is a value determined by an electric field formed by charge carriers accumulated in the layer and has a following relationship:

$$d(1/c^2)/dv = 2/(e\epsilon_0 e N)$$

in which N is a space charge density, C is an electrostatic capacity per  $1 \text{ cm}^2$  in the charge generating layer, V is a bias-voltage applied to the charge generating layer, e is a charge amount of an electron,  $\epsilon$  is a dielectric constant in the charge generating layer, and  $\epsilon_0$  is a vacuum dielectric constant

- 15 As the value of the space charge density is larger, more charge carriers accumulate in the layer. Accordingly the space charge density is adjusted to  $1 \times 10^{16} \text{ cm}^{-3}$  or less in the present invention. Thereby few electrical charges accumulate in the charge generating layer even after repetition use.
- 20 Charging properties are stable. The space charge density can be given according to, for example, a low-frequency C-V method described by Allen J. Twarowsky and A. C. Albecht, J. Chem. Phys. 70, 2255 (1975).

- 25 As above mentioned, a laminated-type photosensitive member which can achieve the objects of the present invention can be provided when a photosensitive layer is formed on an electrically conductive substrate of a small size so that a charge transporting material and a binder resin may be selected to satisfy the relationship of the formula [I]. When 30 a charge generating material and a binder resin are selected so that the mobility and the space charge density may be within a specified range in the charge generating layer, a photosensitive member having stable charging properties even after repetition use can be provided. The present 35 invention is more effective for a photosensitive member of a laminated type having a charge generating layer and a charge transporting layer on an electrically conductive substrate in this order. Further the present invention is effective to be applied to such a copying system as electrostatic latent 40 images are formed on an identical position of the photosensitive member at a 0.5 sec or less interval, particularly 0.3 sec or less interval.

- 45 A laminated type photosensitive member having a charge generating layer and a charge transporting layer on an electrically conductive substrate is explained in detail hereinafter.

- In preparing a photosensitive member of a laminated type, a charge generating material may be deposited in vacuo on an electrically conductive substrate, or a solution containing 50 a charge generating material dissolved in an adequate solvent or a solution containing a pigment and, if necessary, a binder resin dissolved or dispersed in an adequate solvent may be applied onto a substrate and dried. Thus a charge generating layer is formed.

- 55 Then a solution containing a charge transporting material and a binder resin is applied onto the charge generating layer to form a charge transporting layer. The coating of the charge generating layer and the charge transporting layer may be carried out by use of a conventional apparatus such 60 as an applicator, a spray coater, a bar coater, a dipping coater, a roll coater and an doctor blade.

- The charge generating layer is formed to have a layer thickness of 0.01 to 2  $\mu\text{m}$ , preferably 0.1 to 1  $\mu\text{m}$ . The charge generating material is contained in the charge generating 65 layer at an amount of 0.1 to 10 parts by weight, preferably 0.2 to 5 parts by weight on the basis of 1 part be weight of the binder resin. If the amount is too low, sensitivity is poor.

If the amount is too high, chargeability is poor and mechanical strength is low.

A charge generating material useful for the present photosensitive layer is exemplified by organic pigments or dyes, such as bisazo pigments, triarylmethane dyes, thiazine dyes, oxazine dyes, xanthene dyes, cyanine coloring agents, styryl coloring agents, pyrylium dyes, azo dyes, quinacridone pigments, indigo pigments, perylene pigments, polycyclic quinone pigments, bisbenzimidazole pigments, indanthrone pigments, squalylium pigments and phthalocyanine pigments. Any other material is also usable insofar as it generates charge carriers very efficiently upon adsorption of light. In particular, bisazo pigments and phthalocyanine pigments are preferable.

Specific examples of the binder resins used with the charge generating material are thermoplastic resins such as saturated polyesters, polyamides, acrylic resins, ethylene-vinyl acetate copolymers, ion cross-linked olefin copolymers (ionomers), styrene-butadiene block copolymers, polyarylates, polycarbonates, vinyl chloride-vinyl acetate copolymers, cellulose esters, polyimides, styrol resins, polyacetals, phenoxy resins and other similar resins; thermosetting resins such as epoxy resins, urethane resins, silicone resins, phenolic resins, melamine resins, xylene resins, alkyd resins, thermosetting acrylic resins and other similar resins; photocuring resins; photoconductive resins such as poly(N-vinyl carbazoles), poly(vinyl pyrenes), poly(vinyl anthracenes) and other similar resins. Any of these resins may be used singly or in combination with other resins.

The above charge generating materials are dissolved or dispersed together with the above resin in an organic solvent, for example, alcohols such as methanol, ethanol and isopropanol, ketones such as acetone, methyl ethyl ketone and cyclohexanone, amides such as N,N-dimethyl formamide, N,N-dimethyl acetamide, sulfoxides such as dimethyl sulfoxide, ethers such as tetrahydrofuran, dioxane and ethylene glycol monomethyl ether, esters such as methyl acetate and ethyl acetate, aliphatic halogenated hydrocarbons such as chloroform, methylene chloride, dichloroethylene, carbon tetrachloride and trichloroethylene, and aromatic hydrocarbons such as benzene, toluene, xylene, ligroin, monochlorobenzene and dichlorobenzene.

The obtained solution is applied onto an electrically conductive substrate, followed by drying, to form a charge generating layer.

An electrically conductive substrate useful in the present invention may be exemplified by a sheet or drum made of metal or alloy such as copper, aluminum, silver, iron and nickel; a substrate such as a plastic film on which the foregoing metal or alloy is adhered by a vacuum-deposition method or an electroless plating method and the like; a substrate such as a plastic film and paper on which an electroconductive layer is formed by applying or depositing electroconductive polymer, indium oxide, tin oxide etc. Generally, a cylindrical substrate is used. For example, a cut pipe in which an aluminum pipe which is processed by a pultrusion process after an extrusion process is cut and a about a 0.2-0.3 mm thickness portion of the outer surface of the pipe is cut off by means of a cutting apparatus, such as a diamond bit; a DI pipe in which an aluminum disk is deep-drawn to have a cup-like shape and then the outer surface is finished by ironing; an EI pipe in which an aluminum disk is impact-processed to have a cup-like shape and then the outer surface is finished by ironing; and an ED pipe in which aluminum is cold-drawn after an extrusion

process; may be used. The surfaces of these pipes above mentioned may be further cut.

A charge transporting layer is formed on the charge generating layer to have a layer thickness of 27 to 70  $\mu\text{m}$ , preferably 30 to 60  $\mu\text{m}$ . The charge transporting material is contained in the charge transporting layer at an amount of 0.02 to 2 parts by weight, preferably 0.5 to 1.2 parts by weight on the basis of 1 part by weight of the binder resin. If the amount is too low, sensitivity is poor. If the amount is too high, chargeability is poor and mechanical strength of the photosensitive layer is low.

A charge transporting material useful for the preparation of the charge transporting layer is exemplified by hydrazone compounds, pyrazoline compounds, styryl compounds,

15 triphenyl methane compounds, oxadiazole compounds, carbazole compounds, stilbene compounds, enamine compounds, oxazole compounds, triphenylamine compounds, tetraphenyl benzidine compounds and azine compounds. More particularly, 20 p-diphenyaminobenzaldehyde-N,N-diphenyl hydrazone, 2-methyl-4-N,N-diphenylamino- $\beta$ -phenylstilbene,  $\alpha$ -phenyl-4-N,N-diphenylaminostilbene,  $\alpha$ -phenyl-4-N-phenyl-N-p-tolylvinylphenylaminostilbene and 1,1,4,4-bisdiethylaminotetraphenylbutadiene may be used. Polysilanes and other organic glass may be used. The charge transporting materials as above mentioned may be singly or in combination with other materials.

Specific examples of the binder resins used together with the charge transporting material are thermoplastic resins

30 such as saturated polyesters, polyamides, acrylic resins, ethylene-vinyl acetate copolymers, ion cross-linked olefin copolymers (ionomers), styrene-butadiene block copolymers, polyarylates, polycarbonates, vinyl chloride-vinyl acetate copolymers, cellulose esters, polyimides, styrol resins, polyacetals, phenoxy resins and other similar resins; thermosetting resins such as epoxy resins, urethane resins, silicone resins, phenolic resins, melamine resins, xylene resins, alkyd resins, thermosetting acrylic resins and other similar resins; photocuring resins; photoconductive resins 40 such as poly(N-vinyl carbazoles), poly(vinyl pyrenes), poly(vinyl anthracenes) and other similar resins. Any of these resins may be used singly or in combination with other resins.

A solvent which is used for the preparation of the charge 45 transporting layer may be exemplified by an aromatic solvent such as benzene, toluene, xylene and chlorobenzene, a ketone such as acetone, methyl ethyl ketone and cyclohexanone, an alcohol such as methanol, ethanol and isopropanol, an ester such as ethyl acetate and ethyl

50 Cellosolve, a halogenated hydrocarbon such as carbon tetrachloride, carbon tetrabromide, chloroform, dichloromethane and tetrachloroethane, an ether such as tetrahydrofuran and dioxane, an amide such as dimethyl formamide, dimethyl sulfoxide and diethyl formamide.

55 These solvents may be used singly or in combination with other solvents.

Further the photosensitive layer may contain other conventional additives in order to improve coatability and flexibility or to restrain the accumulation of residual potential.

The photosensitive member of the present invention permits, in combination with the binder resin, the use of a plasticizer such as halogenated paraffin, polybiphenyl chloride, dimethyl naphthalene, dibutyl phthalate and o-terphenyl, the use of an electron-attracting sensitizer such as chloranyl, tetracyanoquinodimethane, tetracyanoethylene, trinitro-fluorenone,

dicyanobenzoquinone, tetrachlorophthalic anhydride, and 3,5-dinitrobenzoic acid, or the use of a sensitizer such as methyl violet, rhodamine B, cyanine dyes, pyrylium salts and thiapyrylium salts.

The photosensitive layer may contain an antioxidant in order to prevent deterioration caused by ozone. The antioxidant is exemplified by hindered phenol, hindered amine, paraphenylene diamine, hydroquinone, spirochroman, spiroindanone, hydroquinoline, a derivative thereof, organic phosphine compounds, and organic sulfur compounds.

The antioxidant is contained at an amount of 0.1 to 100 parts by weight, preferably 1 to 50 parts by weight, more preferably 5 to 30 parts by weight on the basis of 100 parts by weight of the charge transporting material.

A photosensitive member of the present invention may have an intermediate layer between the electrically conductive substrate and the photosensitive layer. Thereby, the improvement of adhesivity and coatability, the protection of the substrate and the restraint of charge injection into the photosensitive layer from the substrate can be achieved.

A material useful for forming the intermediate layer is exemplified by polyimides, polyamides, nitrocelluloses, poly(vinyl butyral), poly(vinyl alcohol) and other similar compounds. A desirable thickness of the layer is 1  $\mu\text{m}$  or less. A material having a low electrical resistance may be dispersed in the intermediate layer.

organic layer may contain an oxygen atom, a nitrogen atom, a halogen atom, and an atom in group III or V of the periodic table, if necessary.

5 A photosensitive member of the present invention may be applied, for example, not only to a copying machine but also to a printer or a facsimile which is equipped with a light source, such as a laser, a light emitting diode (LED), a LCD 10 shutter and a Braun tube.

The present invention is further explained with reference to specific examples. It is, of course, not the intention hereby to limit the scope of the invention. In the examples, the term 15 "part(s)" means "part(s) by weight" in so far as it is not explained particularly.

## EXAMPLES 1 AND 2

20

As an electrically conductive substrate, a small aluminum drum having 26 mm diameter and 320 mm length was used in this example.

25

An azo compound represented by the following chemical formula:



A photosensitive member of the present invention may have a surface protective layer. A material useful for forming the surface protective layer is exemplified by acrylic resins, polyaryl resins, polycarbonate resins, urethane resins, thermosetting resins, photocuring resins. These polymers may be used singly. A material of low electrical resistance, such as tin oxide, indium oxide and other similar compounds may be dispersed in the surface protective layer. A desirable thickness of the surface protective layer is 5  $\mu\text{m}$  or less.

45 of 1 part, a polyester resin (Vylon 200; made by Toyo Boseki K.K.) of 1 part were dispersed in hexanone of 500 parts in a sand mill.

The obtained dispersion solution was diluted with tetrahydrofuran of 500 parts and applied onto the aluminum drum. Thus a charge generating layer was formed so that a thickness of the charge generating layer would be about 0.3  $\mu\text{m}$  after drying.

50 Then a diamino compound represented by the following chemical formula:



65 A plasma-polymerized organic layer may be applied to the surface protective layer. The plasma-polymerized

of 50 parts, bisphenol Z polycarbonate of 50 parts, a cyano compound represented by the following formula:



of 1.5 parts and di-ter-butyl-hydroxy-toluene of 4 parts were dissolved in dichloromethane. The obtained solution was applied onto the charge generating layer by a dipping method. Thus a charge transporting layer was formed so that a thickness of the charge transporting layer would be 30  $\mu\text{m}$  (Example 1) or 40  $\mu\text{m}$  (Example 2). Thus laminated type photosensitive members were obtained.

of 1.5 parts and di-ter-butyl-hydroxy-toluene of 4 parts were dissolved in 1,4-dioxane. The obtained solution was applied onto the charge generating layer by a dipping method. Thus a charge transporting layer was formed so that a thickness of the charge transporting layer would be 28  $\mu\text{m}$  (Example 3), 35  $\mu\text{m}$  (Example 4) or 43  $\mu\text{m}$  (Example 5). Thus laminated type photosensitive members were obtained.

### EXAMPLES 3 TO 5

As an electrically conductive substrate, a small aluminum drum having 45 mm diameter and 340 mm length was used in this example.

An azo compound represented by the following chemical formula:



of 1 part, a phenoxy resin (pkHH; made by Union Carbide K.K.) of 0.5 parts and a poly-vinylbutyral resin (#6000; made by Denka Kogyo K.K.) of 0.5 parts were dispersed in cyclohexanone of 500 parts in a sand mill. The obtained dispersion solution was diluted with 1,4-dioxane of 500 parts and applied onto the aluminum drum. Thus a charge generating layer was formed so that a thickness of the charge generating layer would be about 0.4  $\mu\text{m}$  after drying.

Then a distyryl compound represented by the following chemical formula:



of 50 parts, bisphenol C polycarbonate of 60 parts, a cyano compound represented by the following formula:

### EXAMPLE 6

As an electrically conductive substrate, a small aluminum drum having 40 mm diameter and 300 mm length was used in this example.

An azo compound represented by the following chemical formula:



1 part, a phenoxy resin (PKHH; made by Union Carbide K.K.) of 0.5 parts and a poly-vinylbuthyral resin (BX-1; made by Sekisui Kagaku K.K.) of 0.5 parts were dispersed in cyclohexanone of 500 parts in a sand mill for 24 hours. The obtained dispersion solution was diluted with 1,4-dioxane of 500 parts and applied onto the aluminum drum. Thus a charge generating layer was formed so that a thickness of the charge generating layer would be about 0.2  $\mu\text{m}$  after drying.

Then a diamino compound represented by the following chemical formula:



of 50 parts, polycarbonate of bisphenol Z type of 50 parts, a dicyano compound represented by the following formula:

20  
25  
30  
35  
40

of 1.5 parts and di-ter-butyl-hydroxy-toluene of 4 parts were dissolved in dichloromethane. The obtained solution was applied onto the charge generating layer by a dipping method. Thus a charge transporting layer was formed so that a thickness of the charge transporting layer would be 35  $\mu\text{m}$ . Thus a laminated type photosensitive member was obtained.

#### EXAMPLE 7

As an electrically conductive substrate, a small aluminum drum having 40 mm diameter and 300 mm length was used in this example.

40  
45  
50  
55  
60  
65  
70  
75  
80  
85  
90  
95  
100  
105  
110  
115  
120  
125  
130  
135  
140  
145  
150  
155  
160  
165  
170  
175  
180  
185  
190  
195  
200  
205  
210  
215  
220  
225  
230  
235  
240  
245  
250  
255  
260  
265  
270  
275  
280  
285  
290  
295  
300  
305  
310  
315  
320  
325  
330  
335  
340  
345  
350  
355  
360  
365  
370  
375  
380  
385  
390  
395  
400  
405  
410  
415  
420  
425  
430  
435  
440  
445  
450  
455  
460  
465  
470  
475  
480  
485  
490  
495  
500  
505  
510  
515  
520  
525  
530  
535  
540  
545  
550  
555  
560  
565  
570  
575  
580  
585  
590  
595  
600  
605  
610  
615  
620  
625  
630  
635  
640  
645  
650  
655  
660  
665  
670  
675  
680  
685  
690  
695  
700  
705  
710  
715  
720  
725  
730  
735  
740  
745  
750  
755  
760  
765  
770  
775  
780  
785  
790  
795  
800  
805  
810  
815  
820  
825  
830  
835  
840  
845  
850  
855  
860  
865  
870  
875  
880  
885  
890  
895  
900  
905  
910  
915  
920  
925  
930  
935  
940  
945  
950  
955  
960  
965  
970  
975  
980  
985  
990  
995  
1000  
1005  
1010  
1015  
1020  
1025  
1030  
1035  
1040  
1045  
1050  
1055  
1060  
1065  
1070  
1075  
1080  
1085  
1090  
1095  
1100  
1105  
1110  
1115  
1120  
1125  
1130  
1135  
1140  
1145  
1150  
1155  
1160  
1165  
1170  
1175  
1180  
1185  
1190  
1195  
1200  
1205  
1210  
1215  
1220  
1225  
1230  
1235  
1240  
1245  
1250  
1255  
1260  
1265  
1270  
1275  
1280  
1285  
1290  
1295  
1300  
1305  
1310  
1315  
1320  
1325  
1330  
1335  
1340  
1345  
1350  
1355  
1360  
1365  
1370  
1375  
1380  
1385  
1390  
1395  
1400  
1405  
1410  
1415  
1420  
1425  
1430  
1435  
1440  
1445  
1450  
1455  
1460  
1465  
1470  
1475  
1480  
1485  
1490  
1495  
1500  
1505  
1510  
1515  
1520  
1525  
1530  
1535  
1540  
1545  
1550  
1555  
1560  
1565  
1570  
1575  
1580  
1585  
1590  
1595  
1600  
1605  
1610  
1615  
1620  
1625  
1630  
1635  
1640  
1645  
1650  
1655  
1660  
1665  
1670  
1675  
1680  
1685  
1690  
1695  
1700  
1705  
1710  
1715  
1720  
1725  
1730  
1735  
1740  
1745  
1750  
1755  
1760  
1765  
1770  
1775  
1780  
1785  
1790  
1795  
1800  
1805  
1810  
1815  
1820  
1825  
1830  
1835  
1840  
1845  
1850  
1855  
1860  
1865  
1870  
1875  
1880  
1885  
1890  
1895  
1900  
1905  
1910  
1915  
1920  
1925  
1930  
1935  
1940  
1945  
1950  
1955  
1960  
1965  
1970  
1975  
1980  
1985  
1990  
1995  
2000  
2005  
2010  
2015  
2020  
2025  
2030  
2035  
2040  
2045  
2050  
2055  
2060  
2065  
2070  
2075  
2080  
2085  
2090  
2095  
2100  
2105  
2110  
2115  
2120  
2125  
2130  
2135  
2140  
2145  
2150  
2155  
2160  
2165  
2170  
2175  
2180  
2185  
2190  
2195  
2200  
2205  
2210  
2215  
2220  
2225  
2230  
2235  
2240  
2245  
2250  
2255  
2260  
2265  
2270  
2275  
2280  
2285  
2290  
2295  
2300  
2305  
2310  
2315  
2320  
2325  
2330  
2335  
2340  
2345  
2350  
2355  
2360  
2365  
2370  
2375  
2380  
2385  
2390  
2395  
2400  
2405  
2410  
2415  
2420  
2425  
2430  
2435  
2440  
2445  
2450  
2455  
2460  
2465  
2470  
2475  
2480  
2485  
2490  
2495  
2500  
2505  
2510  
2515  
2520  
2525  
2530  
2535  
2540  
2545  
2550  
2555  
2560  
2565  
2570  
2575  
2580  
2585  
2590  
2595  
2600  
2605  
2610  
2615  
2620  
2625  
2630  
2635  
2640  
2645  
2650  
2655  
2660  
2665  
2670  
2675  
2680  
2685  
2690  
2695  
2700  
2705  
2710  
2715  
2720  
2725  
2730  
2735  
2740  
2745  
2750  
2755  
2760  
2765  
2770  
2775  
2780  
2785  
2790  
2795  
2800  
2805  
2810  
2815  
2820  
2825  
2830  
2835  
2840  
2845  
2850  
2855  
2860  
2865  
2870  
2875  
2880  
2885  
2890  
2895  
2900  
2905  
2910  
2915  
2920  
2925  
2930  
2935  
2940  
2945  
2950  
2955  
2960  
2965  
2970  
2975  
2980  
2985  
2990  
2995  
3000  
3005  
3010  
3015  
3020  
3025  
3030  
3035  
3040  
3045  
3050  
3055  
3060  
3065  
3070  
3075  
3080  
3085  
3090  
3095  
3100  
3105  
3110  
3115  
3120  
3125  
3130  
3135  
3140  
3145  
3150  
3155  
3160  
3165  
3170  
3175  
3180  
3185  
3190  
3195  
3200  
3205  
3210  
3215  
3220  
3225  
3230  
3235  
3240  
3245  
3250  
3255  
3260  
3265  
3270  
3275  
3280  
3285  
3290  
3295  
3300  
3305  
3310  
3315  
3320  
3325  
3330  
3335  
3340  
3345  
3350  
3355  
3360  
3365  
3370  
3375  
3380  
3385  
3390  
3395  
3400  
3405  
3410  
3415  
3420  
3425  
3430  
3435  
3440  
3445  
3450  
3455  
3460  
3465  
3470  
3475  
3480  
3485  
3490  
3495  
3500  
3505  
3510  
3515  
3520  
3525  
3530  
3535  
3540  
3545  
3550  
3555  
3560  
3565  
3570  
3575  
3580  
3585  
3590  
3595  
3600  
3605  
3610  
3615  
3620  
3625  
3630  
3635  
3640  
3645  
3650  
3655  
3660  
3665  
3670  
3675  
3680  
3685  
3690  
3695  
3700  
3705  
3710  
3715  
3720  
3725  
3730  
3735  
3740  
3745  
3750  
3755  
3760  
3765  
3770  
3775  
3780  
3785  
3790  
3795  
3800  
3805  
3810  
3815  
3820  
3825  
3830  
3835  
3840  
3845  
3850  
3855  
3860  
3865  
3870  
3875  
3880  
3885  
3890  
3895  
3900  
3905  
3910  
3915  
3920  
3925  
3930  
3935  
3940  
3945  
3950  
3955  
3960  
3965  
3970  
3975  
3980  
3985  
3990  
3995  
4000  
4005  
4010  
4015  
4020  
4025  
4030  
4035  
4040  
4045  
4050  
4055  
4060  
4065  
4070  
4075  
4080  
4085  
4090  
4095  
4100  
4105  
4110  
4115  
4120  
4125  
4130  
4135  
4140  
4145  
4150  
4155  
4160  
4165  
4170  
4175  
4180  
4185  
4190  
4195  
4200  
4205  
4210  
4215  
4220  
4225  
4230  
4235  
4240  
4245  
4250  
4255  
4260  
4265  
4270  
4275  
4280  
4285  
4290  
4295  
4300  
4305  
4310  
4315  
4320  
4325  
4330  
4335  
4340  
4345  
4350  
4355  
4360  
4365  
4370  
4375  
4380  
4385  
4390  
4395  
4400  
4405  
4410  
4415  
4420  
4425  
4430  
4435  
4440  
4445  
4450  
4455  
4460  
4465  
4470  
4475  
4480  
4485  
4490  
4495  
4500  
4505  
4510  
4515  
4520  
4525  
4530  
4535  
4540  
4545  
4550  
4555  
4560  
4565  
4570  
4575  
4580  
4585  
4590  
4595  
4600  
4605  
4610  
4615  
4620  
4625  
4630  
4635  
4640  
4645  
4650  
4655  
4660  
4665  
4670  
4675  
4680  
4685  
4690  
4695  
4700  
4705  
4710  
4715  
4720  
4725  
4730  
4735  
4740  
4745  
4750  
4755  
4760  
4765  
4770  
4775  
4780  
4785  
4790  
4795  
4800  
4805  
4810  
4815  
4820  
4825  
4830  
4835  
4840  
4845  
4850  
4855  
4860  
4865  
4870  
4875  
4880  
4885  
4890  
4895  
4900  
4905  
4910  
4915  
4920  
4925  
4930  
4935  
4940  
4945  
4950  
4955  
4960  
4965  
4970  
4975  
4980  
4985  
4990  
4995  
5000  
5005  
5010  
5015  
5020  
5025  
5030  
5035  
5040  
5045  
5050  
5055  
5060  
5065  
5070  
5075  
5080  
5085  
5090  
5095  
5100  
5105  
5110  
5115  
5120  
5125  
5130  
5135  
5140  
5145  
5150  
5155  
5160  
5165  
5170  
5175  
5180  
5185  
5190  
5195  
5200  
5205  
5210  
5215  
5220  
5225  
5230  
5235  
5240  
5245  
5250  
5255  
5260  
5265  
5270  
5275  
5280  
5285  
5290  
5295  
5300  
5305  
5310  
5315  
5320  
5325  
5330  
5335  
5340  
5345  
5350  
5355  
5360  
5365  
5370  
5375  
5380  
5385  
5390  
5395  
5400  
5405  
5410  
5415  
5420  
5425  
5430  
5435  
5440  
5445  
5450  
5455  
5460  
5465  
5470  
5475  
5480  
5485  
5490  
5495  
5500  
5505  
5510  
5515  
5520  
5525  
5530  
5535  
5540  
5545  
5550  
5555  
5560  
5565  
5570  
5575  
5580  
5585  
5590  
5595  
5600  
5605  
5610  
5615  
5620  
5625  
5630  
5635  
5640  
5645  
5650  
5655  
5660  
5665  
5670  
5675  
5680  
5685  
5690  
5695  
5700  
5705  
5710  
5715  
5720  
5725  
5730  
5735  
5740  
5745  
5750  
5755  
5760  
5765  
5770  
5775  
5780  
5785  
5790  
5795  
5800  
5805  
5810  
5815  
5820  
5825  
5830  
5835  
5840  
5845  
5850  
5855  
5860  
5865  
5870  
5875  
5880  
5885  
5890  
5895  
5900  
5905  
5910  
5915  
5920  
5925  
5930  
5935  
5940  
5945  
5950  
5955  
5960  
5965  
5970  
5975  
5980  
5985  
5990  
5995  
6000  
6005  
6010  
6015  
6020  
6025  
6030  
6035  
6040  
6045  
6050  
6055  
6060  
6065  
6070  
6075  
6080  
6085  
6090  
6095  
6100  
6105  
6110  
6115  
6120  
6125  
6130  
6135  
6140  
6145  
6150  
6155  
6160  
6165  
6170  
6175  
6180  
6185  
6190  
6195  
6200  
6205  
6210  
6215  
6220  
6225  
6230  
6235  
6240  
6245  
6250  
6255  
6260  
6265  
6270  
6275  
6280  
6285  
6290  
6295  
6300  
6305  
6310  
6315  
6320  
6325  
6330  
6335  
6340  
6345  
6350  
6355  
6360  
6365  
6370  
6375  
6380  
6385  
6390  
6395  
6400  
6405  
6410  
6415  
6420  
6425  
6430  
6435  
6440  
6445  
6450  
6455  
6460  
6465  
6470  
6475  
6480  
6485  
6490  
6495  
6500  
6505  
6510  
6515  
6520  
6525  
6530  
6535  
6540  
6545  
6550  
6555  
6560  
6565  
6570  
6575  
6580  
6585  
6590  
6595  
6600  
6605  
6610  
6615  
6620  
6625  
6630  
6635  
6640  
6645  
6650  
6655  
6660  
6665  
6670  
6675  
6680  
6685  
6690  
6695  
6700  
6705  
6710  
6715  
6720  
6725  
6730  
6735  
6740  
6745  
6750  
6755  
6760  
6765  
6770  
6775  
6780  
6785  
6790  
6795  
6800  
6805  
6810  
6815  
6820  
6825  
6830  
6835  
6840  
6845  
6850  
6855  
6860  
6865  
6870  
6875  
6880  
6885  
6890  
6895  
6900  
6905  
6910  
6915  
6920  
6925  
6930  
6935  
6940  
6945  
6950  
6955  
6960  
6965  
6970  
6975  
6980  
6985  
6990  
6995  
7000  
7005  
7010  
7015  
7020  
7025  
7030  
7035  
7040  
7045  
7050  
7055  
7060  
7065  
7070  
7075  
7080  
7085  
7090  
7095  
7100  
7105  
7110  
7115  
7120  
7125  
7130  
7135  
7140  
7145  
7150  
7155  
7160  
7165  
7170  
7175  
7180  
7185  
7190  
7195  
7200  
7205  
7210  
7215  
7220  
7225  
7230  
7235  
7240  
7245  
7250  
7255  
7260  
7265  
7270  
7275  
7280  
7285  
7290  
7295  
7300  
7305  
7310  
7315  
7320  
7325  
7330  
7335  
7340  
7345  
7350  
7355  
7360  
7365  
7370  
7375  
7380  
7385  
7390  
7395  
7400  
7405  
7410  
7415  
7420  
7425  
7430  
7435  
7440  
7445  
7450  
7455  
7460  
7465  
7470  
7475  
7480  
7485  
7490  
7495  
7500  
7505  
7510  
7515  
7520  
7525  
7530  
7535  
7540  
7545  
7550  
7555  
7560  
7565  
7570  
7575  
7580  
7585  
7590  
7595  
7600  
7605  
7610  
7615  
7620  
7625  
7630  
7635  
7640  
7645  
7650  
7655  
7660  
7665  
7670  
7675  
7680  
7685  
7690  
7695  
7700  
7705  
7710  
7715  
7720  
7725  
7730  
7735  
7740  
7745  
7750  
7755  
7760  
7765  
7770  
7775  
7780  
7785  
7790  
7795  
7800  
7805  
7810  
7815  
7820  
7825  
7830  
7835  
7840  
7845  
7850  
7855  
7860  
7865  
7870  
7875  
7880  
7885  
7890  
7895  
7900  
7905  
7910  
7915  
7920  
7925  
7930  
7935  
7940  
7945  
7950  
7955  
7960  
7965  
7970  
7975  
7980  
7985  
7990  
7995  
8000  
8005  
8010  
8015  
8020  
8025  
8030  
8035  
8040  
8045  
8050  
8055  
8060  
8065  
8070  
8075  
8080  
8085  
8090  
8095  
8100  
8105  
8110  
8115  
8120  
8125  
8130  
8135  
8140  
8145  
8150  
8155  
8160  
8165  
8170  
8175  
8180  
8185  
8190  
8195  
8200  
8205  
8210  
8215  
8220  
8225  
8230  
8235  
8240  
8245  
8250  
8255  
8260  
8265  
8270  
8275  
8280  
8285  
8290  
8295  
8300  
8305  
8310  
8315  
8320  
8325  
8330  
8335  
8340  
8345  
8350  
8355  
8360  
8365  
8370  
8375  
8380  
8385  
8390  
8395  
8400  
8405  
8410  
8415  
8420  
8425  
8430  
8435  
8440  
8445  
8450  
8455  
8460  
8465  
8470  
8475  
8480  
8485  
8490  
8495  
8500  
8505  
8510  
8515  
8520  
8525  
8530  
8535  
8540  
8545  
8550  
8555  
8560  
8565  
8570  
8575  
8580  
8585  
8590  
8595  
8600  
8605  
8610  
8615  
8620  
8625  
8630  
8635  
8640  
8645  
8650  
8655  
8660  
8665  
8670  
8675  
8680  
8685  
8690  
8695  
8700  
8705  
8710  
8715  
8720  
8725  
8730  
8735  
8740  
8745  
8750  
8755  
8760  
8765  
8770  
8775  
8780  
8785  
8790  
8795  
8800  
8805  
8810  
8815  
8820  
8825  
8830  
8835  
8840  
8845  
8850  
8855  
8860  
8865  
8870  
8875  
8880  
8885  
8

13

of 1 part, a phenoxy resin (PKHH; made by Union Carbide K.K.) of 0.5 parts and a poly-vinylbutyral resin (BX-1; made by Sekisui Kagaku K.K.) of 0.5 parts were dispersed for 24 hours in cyclohexanone of 500 parts in a sand mill. The obtained dispersion solution was diluted with 1,4-dioxane of 500 parts and applied onto the aluminum drum. Thus a charge generating layer was formed so that a thickness of the charge generating layer would be about 0.2  $\mu\text{m}$  after drying.

Then a diamino compound represented by the following chemical formula:



of 50 parts, polycarbonate of bisphenol Z type of 50 parts, a cyano compound represented by the following formula:



of 1.5 parts and di-ter-butyl-hydroxy-toluene of 4 parts were dissolved in dichloromethane. The obtained solution was applied onto the charge generating layer by a dipping method. Thus a charge transporting layer was formed so that a thickness of the charge transporting layer would be 35  $\mu\text{m}$ . Thus a laminated type photosensitive member was obtained.

#### EXAMPLES 8 AND 9

A photosensitive member was prepared in a manner similar to Example 7 except that a layer thickness of the charge transporting layer was 40  $\mu\text{m}$  (Example 8) or 45  $\mu\text{m}$  (Example 9).

#### EXAMPLE 10

Titanylphthalocyanine of m-type of 0.5 parts, a poly(vinyl butyral) resin (6000C; made by Denki Kagaku Kogyo K.K.)

5,747,208  
14

of 0.5 parts were dispersed for 4 hours in tetrahydrofuran (THF) of 500 parts in a sand mill. The obtained dispersion solution was applied onto a small aluminum drum having 45 mm diameter and 340 mm length. Thus a charge generating layer was formed so that a thickness of the charge generating layer would be about 0.15  $\mu\text{m}$  after drying.

Then a distyryl compound represented by the following chemical formula:



of 50 parts, polycarbonate of bisphenol C type of 60 parts, a cyano compound represented by the following formula:



of 1.5 parts and di-ter-butyl-hydroxy-toluene of 4 parts were dissolved in 1,4-dioxane of 500 parts. The obtained solution was applied onto the charge generating layer. Thus a charge transporting layer was formed so that a thickness of the charge transporting layer would be 35  $\mu\text{m}$ . Thus a laminated type photosensitive member having a two-layer photosensitive layer was obtained.

#### EXAMPLES 11 AND 12

A photosensitive member was prepared in a manner similar to Example 9 except that a layer thickness of the charge transporting layer was 43  $\mu\text{m}$  (Example 11) or 50  $\mu\text{m}$  (Example 12).

#### EXAMPLE 13

As an electrically conductive substrate, a small aluminum drum having 30 mm diameter and 280 mm length was used in this example.

An azo compound represented by the following chemical formula:



10

of 1 part, a polyester resin (Vylon 200; made by Toyo Boseki K.K.) of 0.5 parts and a polybutyral resin (BX-1; made by Sekisui Kagaku K.K.) of 0.5 parts were dispersed for 24 hours in cyclohexanone of 500 parts in a sand mill. The obtained dispersion solution was diluted with 1,4-dioxane of 500 parts and applied onto the aluminum drum. Thus a charge generating layer was formed so that a thickness of the charge generating layer would be about 0.3  $\mu\text{m}$  after drying.

15 Then a diamino compound represented by the following chemical formula:



of 50 parts, polycarbonate of bisphenol Z type of 50 parts, a dicyano compound represented by the following formula:



40



45 of 1.5 parts, di-ter-butyl-hydroxy-toluene of 4 parts and m-terphenyl of 5 parts were dissolved in dichloromethane. The obtained solution was applied onto the charge generating layer by a dipping method. Thus a charge transporting layer was formed so that a thickness of the charge transporting layer would be 40  $\mu\text{m}$ . Thus a laminated type photosensitive member was obtained.

#### EXAMPLE 14

A photosensitive member was prepared in a manner similar to Example 13 except that a layer thickness of the charge transporting layer was 50  $\mu\text{m}$ .

#### Comparative Example 1

A photosensitive member was prepared in a manner similar to Example 1 except that a hydrazone compound represented by the following formula:



55

50

55

60

was contained in the charge transporting layer as a charge transporting material.

#### Comparative Example 2

A photosensitive member was prepared in a manner similar to Example 1 except that a hydrazone compound represented by the following formula:

65 A photosensitive member was prepared in a manner similar to Example 1 except that a hydrazone compound represented by the following formula:

was contained in the charge transporting layer as a charge transporting material.

## Comparative Example 3

A photosensitive member was prepared in a manner similar to Example 7 except that a hydrazone compound represented by the following formula:



was contained in the charge transporting layer as a charge transporting material.

## Comparative Example 4

A photosensitive member was prepared in a manner similar to Example 7 except that a hydrazone compound represented by the following formula:



was contained in the charge transporting layer as a charge transporting material.

## Evaluation

The obtained photosensitive members were evaluated by use of a tester for a photosensitive member shown in FIG. 1. While a photosensitive member (6) was revolved at a 200 mm/sec circumferential speed, it was corona-charged by a charger (5) at a -5 KV applying voltage power to measure an initial surface potential ( $V_0$  (V)). Further an exposure amount for half reducing ( $E_{1/2}$  (lux.sec)), a dark decreasing ratio ( $DDR_1$  (%)) and a residual potential ( $V_R$  (V)) were measured. The exposure amount for half reducing is the exposure amount required for the surface potential to be half the value of the initial surface potential. The dark decreasing ratio is the ratio of a reduced charge amount to the initial charge amount after the initially charged photosensitive member is left in the dark for 1 seconds. The residual potential is the one measured after the irradiation by an eraser (3) (50 lux.sec). The results are summarized in Table 1.

TABLE 1

|     | $V_0$ (V) | $E_{1/2}$ (lux.sec) | $DDR_1$ (%) | $V_R$ (V) |
|-----|-----------|---------------------|-------------|-----------|
| Ex1 | -660      | 0.6                 | 2.0         | -5        |
| Ex2 | -680      | 0.5                 | 1.8         | -5        |
| Ex3 | -670      | 0.6                 | 2.2         | -2        |
| Ex4 | -680      | 0.5                 | 1.7         | -5        |
| Ex5 | -680      | 0.5                 | 1.5         | -7        |
| Ex6 | -675      | 0.8                 | 2.1         | -9        |

TABLE 1-continued

|    |      | $V_0$ (V) | $E_{1/2}$ (lux.sec) | $DDR_1$ (%) | $V_R$ (V) |
|----|------|-----------|---------------------|-------------|-----------|
| 5  | CE1  | -700      | 3.2                 | 1.6         | -70       |
|    | CE2  | -670      | 0.7                 | 2.1         | -20       |
|    | Ex7  | -670      | 0.6                 | 2.0         | -2        |
|    | Ex8  | -680      | 0.5                 | 1.8         | -5        |
|    | Ex9  | -690      | 0.4                 | 1.5         | -5        |
|    | Ex10 | -660      | 0.7                 | 2.3         | -3        |
|    | Ex11 | -675      | 0.6                 | 1.9         | -5        |
|    | Ex12 | -690      | 0.4                 | 1.6         | -7        |
|    | Ex13 | -680      | 0.5                 | 2.0         | -3        |
|    | Ex14 | -690      | 0.4                 | 1.4         | -6        |
| 10 | CE3  | -690      | 3.4                 | 1.6         | -65       |
|    | CE4  | -670      | 0.8                 | 2.3         | -35       |

Ex: Example  
CE: Comparative Example

With respect to Examples 1 to 6 and Comparative Examples 1 and 2, a mobility of electrical charges in the photosensitive member was measured at 25° C. by the time of flight method. The results are summarized in Table 2.

TABLE 2

|    |     | A     | B     |
|----|-----|-------|-------|
| 25 | Ex1 | 0.08  | -4.70 |
|    | Ex2 | 0.08  | -4.70 |
|    | Ex3 | 0.09  | -4.88 |
|    | Ex4 | 0.09  | -4.88 |
|    | Ex5 | 0.09  | -4.88 |
|    | Ex6 | 0.11  | -5.32 |
|    | CE1 | 0.155 | -6.52 |
|    | CE2 | 0.131 | -5.89 |

Ex: Example  
CE: Comparative Example  
35 A and B are the same as explained in the formula [I]

The photosensitive members of Example 1 and Comparative example 1 were subjected to the following durability test. The revolution number of the drum was adjusted so that a time period between an irradiation process and a developing process would be 0.2 seconds. A copying process in which the irradiation power had 2 lux.sec was repeated 1,000 times under L/L environmental conditions (10° C., 35%). An initial surface potential ( $V_0$  (V)), a potential at an irradiated portion ( $V_i$  (V)) and a residual potential ( $V_R$  (V)) were measured. The results are summarized in Table 3.  $V_0'$  (V),  $V_i'$  (V) and  $V_R'$  (V) in Table 3 represent respectively a value after 1,000 times repetition.

TABLE 3

|    | initial   |           |           | after 1000 times of copy |           |           |
|----|-----------|-----------|-----------|--------------------------|-----------|-----------|
|    | $V_0$ (V) | $V_i$ (V) | $V_R$ (V) | $V_0$ (V)                | $V_i$ (V) | $V_R$ (V) |
| 55 | Ex 1      | -670      | -20       | -10                      | -660      | -20       |
|    | Ex 6      | -675      | -50       | -9                       | -650      | -70       |
|    | CE 1      | -650      | -105      | -50                      | -550      | -210      |

Ex: Example  
CE: Comparative Example

With respect to Examples 7 to 14 and Comparative Examples 3 to 4, a mobility of electrical charges in the charge transporting layer and the charge generating layer was measured similarly as above mentioned. The results are 65 summarized in Table 4. A space charge density was also measured by the C-V method above mentioned. The results are summarized in Table 4.

TABLE 4

|       | Charge generating layer                |                                             | Charge transporting layer  |       |
|-------|----------------------------------------|---------------------------------------------|----------------------------|-------|
|       | Mobility<br>(cm <sup>2</sup> /V · sec) | space charge<br>density (cm <sup>-3</sup> ) | Coefficient of<br>Mobility |       |
|       |                                        |                                             | A                          | B     |
| EX 7  | $1 \times 10^{-7}$                     | $0.7 \times 10^{15}$                        | 0.08                       | -4.70 |
| EX 8  | $1 \times 10^{-7}$                     | $0.7 \times 10^{15}$                        | 0.08                       | -4.70 |
| EX 9  | $1 \times 10^{-7}$                     | $0.7 \times 10^{15}$                        | 0.08                       | -4.70 |
| EX 10 | $3 \times 10^{-7}$                     | $5 \times 10^{15}$                          | 0.09                       | -4.88 |
| EX 11 | $3 \times 10^{-7}$                     | $5 \times 10^{15}$                          | 0.09                       | -4.88 |
| EX 12 | $3 \times 10^{-7}$                     | $5 \times 10^{15}$                          | 0.09                       | -4.88 |
| EX 13 | $5 \times 10^{-7}$                     | $2 \times 10^{15}$                          | 0.08                       | -4.60 |
| EX 14 | $5 \times 10^{-7}$                     | $2 \times 10^{15}$                          | 0.08                       | -4.60 |
| CE 3  | $1 \times 10^{-7}$                     | $0.7 \times 10^{15}$                        | 0.155                      | -6.52 |
| CE 4  | $1 \times 10^{-7}$                     | $0.7 \times 10^{15}$                        | 0.131                      | -5.89 |

Ex: Example

CE: Comparative Example

The photosensitive members of Examples 7, 10 and 13 and Comparative examples 3 and 4 were subjected to the following durability test. The revolution number of the drum was adjusted so that a time period between an irradiation process and a developing process would be 0.2 seconds. A copying process in which the irradiation power had 2 lux.sec was repeated 10,000 times under L/L environmental conditions (10° C., 35%). An initial surface potential ( $V_o$  (V)), a potential at an irradiated portion ( $V_i$  (V)) and a residual potential ( $V_R$  (V)) were measured. The results are summarized in Table 5.  $V_o$ ,  $V_i$  and  $V_R$  in Table 5 represent respectively a value after 10,000 times repetition.

Further the photosensitive members obtained in Example 1 and Example 7 were respectively installed in a copying machine (EP-3150; made by Minolta Camera) and subjected to a durability test with respect to 50,000 times of copy. A lowering of the surface potential was small and excellent copy images could be formed without deterioration of image quality.

TABLE 5

|       | initial      |              | after 10,000 times of copy |              |              |              |
|-------|--------------|--------------|----------------------------|--------------|--------------|--------------|
|       | $V_o$<br>(V) | $V_i$<br>(V) | $V_R$<br>(V)               | $V_o$<br>(V) | $V_i$<br>(V) | $V_R$<br>(V) |
| Ex 7  | -670         | -20          | -5                         | -660         | -20          | -10          |
| Ex 10 | -660         | -30          | -5                         | -640         | -35          | -10          |
| Ex 13 | -680         | -15          | -5                         | -670         | -20          | -15          |
| CE 3  | -690         | -120         | -50                        | -560         | -240         | -120         |
| CE 4  | -670         | -60          | -35                        | -580         | -150         | -80          |

Ex: Example

CE: Comparative Example

What is claimed is:

1. A method for developing an electrostatic latent image formed on a photosensitive member comprising forming an electrostatic latent image on an identical position of a laminated photosensitive member at a 0.5 second or less interval and, developing the electrostatic latent image, wherein the photosensitive member comprises a charge generating layer containing an organic charge generating material, said charge generating layer having a mobility in the charge generating layer of at least  $1 \times 10^{-8}$  cm<sup>2</sup>/V.sec under an electrical field of  $5 \times 10^5$  V/cm and a space charge density of the charge generating layer of  $1 \times 10^{16}$  cm<sup>-3</sup> or less; a charge transporting layer having a thickness of at least 35  $\mu$ m and containing an organic charge transporting material, said charge transporting layer having a mobility ( $\mu$ ) of electrical charges satisfying the following formula:

$$\log \mu = A \times E^{1/2} + B$$

[I]

in which E is an electrical field (V/ $\mu$ m), A represents a value of 0.11 or less and B is -5.9 or more; and a cylindrical substrate having a drum size of 50 mmΦ or less.

2. The method of claim 1, wherein the charge generating layer has a layer thickness of 2  $\mu$ m or less.

3. The method of claim 2, wherein the transporting layer has a thickness in the range of 35-60  $\mu$ m.

4. The method of claim 1, wherein the charge generating layer is formed on the charge transporting layer.

5. The method of claim 1, wherein the charge generating material is contained in the charge generating layer at an amount of 0.1 to 10 parts by weight on the basis of 1 part by weight of a binder resin.

6. The method of claim 1, wherein the charge transporting material is contained in the charge transporting layer at an amount of 0.02 to 2 parts by weight on the basis of 1 part by weight of a binder resin.

7. The method of claim 1, wherein A is 0.1 or less and B is -5 or more.

8. The method of claim 1, wherein the mobility of charges in a charge generating layer is  $5 \times 10^{-8}$  cm<sup>2</sup>/V.sec or more under an electric field of  $5 \times 10^5$  V/sec.

9. The method of claim 1, wherein the charge generating material is selected from the group consisting of bisazo pigments, triarylmethane dyes, thiazine dyes, oxazine dyes, xanthene dyes, cyanine pigments, styryl pigments, pyrilium pigments, azo pigments, quinacridone pigments, indigo pigments, perylene pigments, polycyclic quinone pigments, bisbenzimidazole pigments, indanthrone pigments and squarylium pigments.

10. The method of claim 1, wherein the charge generating material is a trisazo compound of the formula:



11. The method of claim 1, wherein the charge transporting material is selected from the group consisting pyrazoline compounds, styryl compounds, triphenylmethane compounds, oxadiazole compounds, carbazole compounds, stilbene compound, enamine compounds, oxazole compounds, triphenylamine compounds, tetraphenyl benzidine compounds and azine compounds. 15
12. The method of claim 1, wherein the charge transporting material is a styryl compound. 20
13. The method of claim 1, wherein the charge transporting material is a triphenyl compound.

\* \* \* \* \*